

April 29, 1924.

1,492,087

J. F. SHAWHAN

ELECTRICAL SMELTING FURNACE

Original Filed April 15, 1920



## UNITED STATES PATENT OFFICE.

JABEA F. SHAWHAN, OF DAYTON, OHIO, ASSIGNOR OF ONE-HALF TO PERLE L. SAGEBIEL, OF DAYTON, OHIO.

## ELECTRICAL SMELTING FURNACE.

Original application filed April 15, 1920, Serial No. 374,030. Divided and this application filed February 18, 1924. Serial No. 693,505.

*To all whom it may concern:*

Be it known that I, JABEA F. SHAWHAN, a citizen of the United States, and residing at Dayton, State of Ohio, have invented the new and useful Improvement in Electrical Smelting Furnaces, of which the following is a specification.

This invention relates to smelting furnaces, and more particularly to that type of furnace used for smelting pyritic ores. This application is a division of application Serial Number 374,030, filed April 15, 1920.

In the process of pyritic smelting, the heat required for the smelting process is obtained by combustion of materials contained in the ores themselves, particularly sulphur and iron in the case of pyritic ores. In order to carry on such a process, pure air in a heated condition must be supplied to the charge to cause oxidation of the sulphur and iron. The charge can, of course, first be brought to a sufficiently high temperature so that the oxidation will be carried on automatically, by rapid oxidation of the iron and sulphur, but once this condition has been attained, the process goes on of itself so long as the proper supply of heated air and ore is maintained.

One of the objects of this invention, therefore, is to provide a smelting furnace adapted to carry on such a smelting process continuously by providing an adequate supply of properly heated air upon the charge.

In a great many cases, facilities for smelting by ordinary methods are not on hand at the mine and ores must be shipped to a distance to be smelted. As the ores in the mine usually carry only about 10% of their weight in valuable metals, a great saving can be effected by carrying on the smelting operation at the mine, thereby saving the cost of transporting the bulky ores and the necessary fuel for heating the air and the charge. As water power is usually available in mining districts, and when transformed into electrical energy, can be used for heating purposes, this invention provides means for carrying on a smelting process at the mines.

Another object of this invention, therefore, is to provide means for utilizing materials and sources of energy available at or near the mine location for the smelting process.

Another object of this invention is to provide electric means for heating the air used in such a process. 55

Further objects will appear from the detail description taken in connection with the accompanying drawing which represents a 60 sectional view in elevation of a furnace embodying this invention.

Referring now to the drawing, 1 designates the ore stack, 2 is the contracted portion thereof or smelting chamber, and 3 is 65 the crucible. The crucible 3 is provided with an outlet 4 for the slag and an outlet 5 for the matte. Opening into the crucible at the sides are tuyères 6. These may be all of the usual construction, the lower part of 70 the furnace, including the crucible, and the smelting chamber are usually constructed of brick and lined with refractory material, while the ore stack 1 may be of cast iron and may be provided with a water jacket 75 8 to keep it cool.

Underneath the smelting furnace is a chamber 30 in which are mounted electrodes 33, 34, 35 and 36, adapted to form in this case, two arcs for heating this chamber. One, 80 two or more arcs may be used, according to circumstances. These electrodes pass through the walls of the chamber and are insulated by bushings of refractory material 37 and 38. The lower electrodes 33 and 35 85 are provided with connectors 12 for connection to the electric circuit. The upper electrodes 34 and 36 are each provided with an elevating device 39 such as a rack and pinion movement. These electrodes are 90 further equipped with connectors, not shown, for connection to the circuit.

Surrounding the heating chamber 30 is a series of air passages 40 communicating at the lower end with the air heating chamber 95 41 and at the upper end with the tuyères 6. The air supply enters the chamber 14 at the inlet 42 and passes through the ducts 43 to the heating chamber 41 where it is heated by contact with the hot electrodes 33 and 35, 100 passing thence up through the passages 40; being heated by contact with the hot walls 44 of the heating chamber 30, to the tuyères 6. This arc-heated chamber may be put to double use by using it as a refining furnace. 105 To this purpose it may be provided with an inlet 31 and an outlet 32. The material to be operated upon is spread over the floor to

be acted upon by the arc heat. If said material is a conductor of electric current it may be heated by passing the current directly through it.

6 The electrical connections of the furnace to the supply circuit may be made as shown in the drawing. The electrodes are connected through the double throw switch 45 to the secondary of an adjustable transformer 46 connected to the supply line. With this arrangement, the furnace can be used either as an arc furnace or as a resistance furnace. By throwing the switch 45 to the upper position, the electrodes 33 and 15 35 are connected to one side of the circuit and the electrodes 34 and 36 to the other side of the circuit. It is evident that with this connection either or both of the electric furnaces may be used as an arc furnace by 20 touching and separating the electrodes by means of the controlling device 39. It is convenient to use furnace in this way as an arc furnace when starting up on a new charge, as heat can be generated more rapidly. When the charge has melted down, the 25 switch 45 may be thrown to the lower position whereby the electrodes 33 and 35 are connected to opposite sides of the circuit. With this connection, the furnace operates 30 as a resistance furnace establishing a circuit through the molten charge. With this connection, it is immaterial whether the upper electrodes are or are not in contact with the lower electrodes, since each pair is short 35 circuited by the switch 45.

It will be seen, therefore, that this invention provides a combination smelting and refining furnace which is very effective. The heat generated by the current is applied directly to the material to be heated, so that there is no waste and great economy of operation is, therefore, possible. The arrangement of the furnace chambers and air passages is also such as to conserve all 40 the heat possible, so that additional saving is effected. On account of the easy adjustability of the electric current, the application of heat can be closely regulated and the smelting process can, therefore, be very 45 accurately controlled.

It is obvious that various changes may be made in the details of construction without departing from the spirit of this invention; it is, therefore, to be understood that this 50 invention is not to be limited to the specific details shown and described.

Having thus described the invention, what is claimed is:

1. A pyritic smelting furnace, comprising, 60 a furnace chamber adapted to receive the charge and provided with tuyères, means for delivering air to said tuyères, and an enclosed electric arc adapted to heat said air.

2. A pyritic smelting furnace, comprising, 65 a furnace chamber adapted to receive the

charge and provided with tuyères, means for delivering air to said tuyères, and an electric arc adapted to heat said air, but out of contact therewith.

3. A pyritic smelting furnace, comprising, 70 a furnace chamber adapted to receive the charge and provided with tuyères, means for delivering air to said tuyères, and an electric arc adapted to heat said air, without extracting oxygen therefrom. 75

4. A pyritic smelting furnace, comprising, 80 a furnace chamber adapted to receive the charge and provided with tuyères, means for delivering air to said tuyères, and means for heating said air including a heating chamber, an electric arc adapted to heat said chamber, and means for circulating said air over the walls of said chamber adapted to heat said air but out of contact with said arc. 85

5. A pyritic smelting furnace, comprising, 90 a chamber adapted to receive the charge and provided with tuyères, means for delivering air to said tuyères, and means for heating said air including a heating chamber, an electric arc adapted to heat said chamber, and means for circulating said air over the walls of said chamber adapted to heat said air without extracting oxygen therefrom. 95

6. A pyritic smelting furnace, comprising, 100 a smelting chamber adapted to receive a charge and provided with tuyères, means for delivering air to said tuyères, and means for heating said air including an electric arc chamber, and air passages surrounding said chamber and communicating with said tuyères. 105

7. A pyritic smelting furnace, comprising, 110 a smelting chamber adapted to receive a charge and provided with tuyères, means for delivering air to said tuyères, and means for heating said air including an electric arc chamber disposed below said smelting chamber, and air passages surrounding said chamber and communicating with said tuyères. 115

8. A pyritic smelting furnace, comprising, 120 a smelting chamber adapted to receive a charge and provided with tuyères, means for delivering air to said tuyères, and means for heating said air including an arc-heated refining chamber, and air passages surrounding said chamber and communicating with said tuyères. 125

9. A pyritic smelting furnace, comprising, 130 a smelting chamber adapted to receive a charge and provided with tuyères, means for delivering air to said tuyères, and means for heating said air including an arc-heated refining chamber, disposed below said smelting chamber, and air passages surrounding said chamber and communicating with said tuyères.

In testimony whereof I affix my signature this 28 day of February, 1923.

JABEA F. SHAWHAN.